

# UNITED STATES PATENT OFFICE.

FRED KIMBLE, OF PEORIA, ILLINOIS.

## MAKING TARGETS.

SPECIFICATION forming part of Letters Patent No. 334,782, dated January 26, 1886.

Application filed July 23, 1885. Serial No. 172,495. (No specimens.)

*To all whom it may concern:*

Be it known that I, FRED KIMBLE, a citizen of the United States, residing in Peoria, in the county of Peoria and State of Illinois, have invented certain new and useful Improvements in the Art of Making Targets, of which the following is a specification.

My invention relates to that class of targets known as "clay pigeons," "blackbirds," and the like, made, usually, of clay or other fragile material and adapted to be thrown through the air from a suitable trap, to be shot at by marksmen, and has for its object the production of a target which will be fragile, so as to be readily shattered when struck by a pellet of shot, that will not be affected by any atmospheric changes to which it may be subjected, and which will be cheap.

To carry my invention into effect, I take a quantity of pitch obtained by distilling off the light oils from coal-tar, and place it in a suitable vessel over a fire and melt it. I then add to each one hundred pounds of melted pitch from twenty-five to seventy-five pounds of whiting or plaster-of-paris and thoroughly mix by agitation. When this composition is heated to about 400° Fahrenheit, it is poured into suitable molds, where it quickly chills. Before adding either the plaster-of-paris or whiting to the melted pitch I prefer to heat the same, in order to thoroughly dry it and to facilitate the mixing with the pitch. The quantity of plaster-of-paris or whiting (and I

use either at will) used to a given quantity of pitch depends upon the condition of the pitch on being taken from the still. If the pitch is boiled so as to stand a temperature of, say, about 175° before softening and melting, I then use about twenty-five pounds of the plaster-of-paris to one hundred pounds of pitch, and if to 140°, then about seventy-five pounds of the plaster-of-paris or whiting. In other words, the harder the pitch is boiled the less oil there is in it to be absorbed, and the minimum quantity of plaster-of-paris is used, and the softer the pitch the more plaster-of-paris is used.

Targets composed of these materials, pitch and either whiting or plaster-of-paris, when combined and molded as above described, give the very best results, and are not affected by atmospheric changes.

What I claim, and desire to secure by Letters Patent, is—

1. As a new article of manufacture, a target composed of pitch and plaster-of-paris or whiting, in the proportions specified.
2. The process of making targets, which consists in mixing with melted pitch a quantity of either plaster-of-paris or whiting, and then pouring the composition so formed into suitable molds, substantially as described.

FRED KIMBLE.

Witnesses:

EDWARD H. WALKER,  
FRANK JACK.